

Patented Mar. 18, 1924.

1,487,124

# UNITED STATES PATENT OFFICE.

JAMES ROBERT STACK, OF PERTH AMBOY, NEW JERSEY, ASSIGNOR TO AMERICA SMELTING AND REFINING COMPANY, OF NEW YORK, N. Y., A CORPORATION OF NEW JERSEY.

## ELECTROLYTIC PROCESS.

No Drawing. Application filed December 30, 1920, Serial No. 434,114. Renewed January 14, 1924.

To all whom it may concern:

Be it known that I, JAMES ROBERT STACK, a citizen of the United States, and resident of Perth Amboy, in the county of Middlesex and State of New Jersey, have invented certain new and useful Improvements in Electrolytic Processes, of which the following is a specification.

The invention relates to certain new and useful improvements in the production of electrically refined tin from impure tin cast in the form of anodes and to an improved form of electrolyte suitable for the process hereinafter featured.

15 It is suggested in the application of Harry H. Alexander, Serial No. 434,124, filed under even date, that an electrolyte be produced from the impure tin of such a character that it will insure the continued 20 maintenance of the electrolytic deposition of the tin during the refining operation and which will itself be devoid of lead and other detrimental impurities usually present in the tin to be refined. It has been known to 25 use sulphuric acid for the purpose of precipitating the lead present and to use hydrofluosilicic acid to dissolve the tin from the anodes without the formation of the basic salts of tin. In the Alexander application 30 it is suggested that the amount of sulphuric acid be increased over the amount necessary to combine with the lead present and that the amount of hydrofluosilicic acid heretofore used in such electrolytes be correspondingly reduced in amount.

It is further suggested in the application of Clarence P. Linville, Serial No. 434,118, filed under even date, that the electrolyte be improved by the addition of free hydrochloric acid or by sodium chloride in the presence of an excess of sulphuric acid and that the electrolyte may be further improved by the use of certain organic addition agents, such as cresylic acid and glue 45 as more particularly defined in the application of Frank C. Mathers, Serial No. 257,700, filed October 11, 1918.

While these several sulphuric hydrofluosilicic acid electrolytes have given entire 50 satisfaction, in practice they possess the economic disadvantage that hydrofluosilicic acid is expensive to manufacture and is consumed rapidly during the electrolytic operations in which it is employed as a solvent for the tin.

The invention features economy in cost of operation not only in connection with the cost of the reagent materials in the electrolyte but also in the amount of electric current used per unit mass of tin deposited and in the amount of waste material necessary to handle.

Accordingly, one of the objects of the invention is to provide an electrolyte which will possess the desirable characteristics inherent in the electrolytes featured in the above identified applications, such as ready solubility of the anodes, elimination of polarization, continuity of action, and the obtaining of a good deposit of tin which will be smooth, dense and adherent but that these results be affected by the use of a cheaper material than the hydrofluosilicic acid heretofore used.

I attain this phase of the invention by substituting for the hydrofluosilicic acid heretofore used one of the cheap cresol sulphonic acids. It has been found that sulphonic acid can be used in this connection for a dual purpose, first, as an addition agent in place of or in part substitution for the glue and cresylic acid addition agents, and second, to replace the hydrofluosilicic acid, either in whole or in part.

One form of sulphonic acid which has given entire satisfaction is made by sulphonating crude cresylic acid with strong sulphuric acid but it is to be understood that this form of sulphonic acid is merely suggestive.

The sulphonic acid can be prepared from benzol, phenol cresol, and crude cresylic acid; the best results having been obtained with phenol sulphonic acid, cresol sulphonic acid and a mixture of benzol and phenol sulphonic acid.

Addition agents, such as glue and cresylic acid may be used but the amount of these addition agents necessary to effect the desired results has been found to be less than in the former methods where hydrofluosilicic acid was used as the tin solvent. It has also been found in practice that one to two per cent by weight of sulphonic acid is entirely satisfactory when used in connection with hydrofluosilicic acid but in case the latter acid is eliminated an equivalent larger amount of the sulphonic acid is necessary. An amount as high as fifteen per cent by weight of sulphonic acid

has been used with entire satisfaction where the hydrofluosilicic acid has been omitted but ten per cent by weight is suggested in this case.

One form of electrolyte which is at present in use, analyzes as follows:

Tin 4.0% by weight in "ous" form; sulphuric acid ( $H_2SO_4$ ) 5.0% by weight; sulphonic acid 2.0% by weight; hydrofluosilicic acid ( $H_2SiF_6$ ) 2.0% by weight; hydrofluoric acid (HF) 0.6% by weight due to decomposition of  $H_2SiF_6$ ; hydrochloric acid (HCl) 0.2% by weight; sodium sulphate ( $NaSO_4$ ) due to addition of  $NaCl$ ; addition agents glue, cresylic acid, etc.

With the addition of sulphonic acid it is possible to maintain the continuity of the electrolytic process with a smaller percentage of tin in solution than has been known heretofore thus avoiding a possible source of waste in tin lost in the precipitates. It is suggested that about two to four per cent of tin in the "ous" state gives the most satisfactory results and tin in this state has the additional advantage in that reduced power may be used than where the tin is in the "ic" form.

Still featuring economy of production it is required that the least possible amount of electric current be used. As the amperage necessary to effect the operation is theoretically fixed at about eight amperes per square foot of cathode surface, the only possible way to effect a saving in power used, aside from the observing of good electrical practice, is to reduce the voltage. Heretofore when the process was carried on under temperature of 60-70° F. the voltage per tank was  $\frac{1}{2}$  to  $\frac{1}{4}$  volts and only about 50% of the anode was dissolved before adhering slimes prevented further anode corrosion. It is found, however, that the heating of the electrolyte not only improved the process but permitted as much as a fifty per cent drop in voltage necessary. For instance, it was found that the heating of the electrolyte to maintain a temperature of approximately 95° F. had the effect of permitting a drop in voltage to 0.2 to 0.25 volts, thus effecting a material saving in power with resulting cheapness of operation. In addition to this it was possible to dissolve 75% to 80% of the anodes before they became too thin for effective work. Heating of the electrolytic solution was also found to assist in preventing the formation of outgrowths upon the cathode surface and in general a better anode corrosion was maintained, better conductivity was provided and in general an improved deposit was attained.

Having thus described my invention, I claim:

1. In the electrolytic refining of impure tin containing lead, the process of preventing contamination of the tin deposited from

the impure tin anode upon the cathode, which consists in employing as the electrolyte a solution of tin in sulphonic acid and a protective agent sufficient to convert the lead contained in the dissolving tin anode into a compound insoluble in the electrolyte. 70

2. In the electrolytic refining of impure tin containing lead, the process of preventing contamination of the tin deposited from the impure tin anode upon the cathode, which consists in employing as the electrolyte a solution of tin in a mixture of sulphonic and sulphuric acids. 75

3. In the electrolytic refining of impure tin, the process of producing an appropriate electrolyte for the refining operation which consists in passing an electric current of suitable voltage and amperage from the impure tin as an anode to a cathode through a solution containing sulphuric acid to five per cent and sulphonic acid two to four per cent. 80

4. In the electrolytic refining of impure tin containing lead, the process of preventing contamination of the tin deposited from the impure tin anode upon the cathode, which consists in employing as the electrolyte a solution of tin in hydrofluosilicic acid and which contains sulphonic acid. 90

5. In the electrolytic refining of impure tin containing lead, the process of preventing contamination of the tin deposited from the impure tin anode upon the cathode, which consists in employing as the electrolyte a solution of tin in a mixture of sulphonic, sulphuric and hydrofluosilicic acid. 100

6. In the electric refining of impure tin containing lead, the process of preventing contamination of the tin deposited from the impure tin anode upon the cathode, which consists in employing as the electrolyte a solution of tin in a mixture of sulphonic and sulphuric acids and an addition agent. 105

7. In the electrolytic refining of impure tin containing lead, the process of preventing contamination of the tin deposited from the impure tin anode upon the cathode, which consists in employing as the electrolyte a solution of tin in sulphuric acid approximately two to five per cent by weight, sulphonic acid approximately one to two per cent by weight and hydrofluosilicic acid approximately two per cent by weight. 110

8. In the electrolytic refining of impure tin containing lead, the process which consists in employing as the electrolyte a solution of tin, two to four per cent by weight in the "ous" form together with sulphonic acid and a protective agent sufficient to convert the lead present in the electrolyte into a compound insoluble in the same. 115

9. In the electrolytic refining of impure tin containing lead, the process which consists in employing as the electrolyte a solution of tin together with sulphonic acid and

- 5 a protective agent sufficient to convert the lead present in the electrolyte into a compound insoluble in the same and an agent capable of preventing the formation of hard 50 slimes.
- 10 10. An electrolyte for the deposition of tin comprising an electrolytic solution of tin in hydrofluosilicic acid in an amount approximately two to four per cent of tin by 55 weight and containing sulphonic acid.
- 11 11. An electrolyte for the deposition of tin comprising an electrolytic solution of tin in hydrofluosilicic acid in an amount approximately two to four per cent of tin by 60 weight and containing sulphonic acid approximately one to two per cent by weight.
- 12 12. An electrolyte for the deposition of tin free from lead comprising an electrolytic solution of tin in hydrofluosilicic acid approximately two to four per cent of tin by 65 weight and containing a protective agent in an amount sufficient to convert the lead into a compound insoluble in the electrolyte and sulphonic acid.
- 13 13. An electrolyte for the deposition of tin free from lead comprising an electrolytic solution of tin in hydrofluosilicic acid approximately two to four per cent of tin by 70 weight and containing a protective agent in an amount sufficient to convert the lead into a compound insoluble in the electrolyte and sulphonic acid approximately one to two per cent by weight and an addition agent.
- 14 14. An electrolyte containing sulphonic, sulphuric and hydrofluosilicic acids together with an addition agent.
- 15 15. In the electrolytic refining of impure tin containing lead, the process which consists in employing as the electrolyte a solution of tin, two to four per cent by weight in the "ous" form together with sulphonic acid and a protective agent sufficient to convert the lead present in the electrolyte into a compound insoluble in the same and an agent capable of forming hydrochloric acid under the conditions present.
- 16 16. In the electrolytic refining of impure tin containing lead, the process which consists in employing as the electrolyte a solution of tin, two to four per cent by weight in the "ous" form together with sulphuric acid in excess of the amount sufficient to convert the lead present into an insoluble compound and a halogen salt capable of reacting with the excess of sulphuric acid to form a free halogen acid.
- 17 17. In the electrolytic refining of impure tin containing lead, the process which consists in employing as the electrolyte a solution of tin, two to four per cent by weight in the "ous" form together with sulphuric acid in excess of the amount sufficient to convert the lead present into an insoluble compound and a sodium chloride.
- 18 18. An electrolyte for the deposition of tin free from lead comprising a solution of tin in hydrofluosilicic acid, and containing sulphuric acid in an amount in excess of the amount necessary to precipitate the lead present, a halogen salt capable of reacting with the excess of sulphuric acid to form a free halogen acid, sulphonic acid and an addition agent.
- 19 19. An electrolyte for the deposition of tin free from lead comprising a solution of tin in hydrofluosilicic acid and containing sulphuric acid in an amount in excess of the amount necessary to precipitate the lead present, a halogen salt capable of reacting with the excess of sulphuric acid to form a free halogen acid and an addition agent.
- 20 20. In the electrolytic refining of impure tin containing lead, the method of producing an appropriate electrolyte for the refining operation, which consists in passing an electric current of suitable voltage and amperage from the impure tin as an anode to a cathode through an electrolyte which is a solvent of tin and lead, and protecting the electrolyte from contamination by lead, by incorporating with the electrolyte an agent which will combine with the lead to form an insoluble compound together with sulphonic acid while subjecting the electrolyte to a temperature higher than room temperature.
- 21 21. In the electrolytic refining of impure tin containing lead, the method of producing an appropriate electrolyte for the refining operation, which consists in passing an electric current of suitable voltage and amperage from the impure tin as an anode to a cathode through an electrolyte which is a solvent of tin and lead, and protecting the electrolyte from contamination by lead, by incorporating with the electrolyte an agent which will combine with the lead to form an insoluble compound together with sulphonic acid while subjecting the electrolyte to a temperature approximately 95° F.
- 22 22. In the electrolytic refining of impure tin containing lead, the method of producing an appropriate electrolyte for the refining operation which consists in passing an electric current at approximately 0.2 to 0.25 volts from the impure tin as an anode to a cathode through an electrolyte protecting the electrolyte from contamination by lead and heating the electrolyte during the passage of the electric current.
- 23 23. In the electrolytic refining of impure tin containing lead, the method of producing an appropriate electrolyte for the refining operation which consists in passing an electric current at approximately 0.2 to 0.25 volts from the impure tin as an anode to a cathode through an electrolyte containing sulphonic acid, protecting the electro-

lyte from contamination by lead and heating the electrolyte during the passage of the electric current.

24. In the electrolytic refining of impure 5 tin containing lead, the method of producing an appropriate electrolyte for the refining operation, which consists in passing an electric current at approximately 0.2 to 0.25 volts from the impure tin as an 10 anode to a cathode through an electrolyte containing sulphonic and sulphuric acid and heating the electrolyte during the electrolytic action.

25. In the electrolytic refining of impure 15 tin containing lead, the method of producing an appropriate electrolyte for the refining operation, which consists in passing an electric current at approximately 0.2 to 0.25 volts from the impure tin as an 20 anode to a cathode through an electrolyte containing sulphonic hydrofluosilicic acid and sulphuric acid and heating the electrolyte during the electrolytic action.

26. In the electrolytic refining of impure 25 tin containing lead, the method of producing an appropriate electrolyte for the refining operation, which consists in passing an electric current at approximately 0.2 to 0.25 volts from the impure tin as an 30 anode to a cathode through an electrolyte containing sulphonic and sulphuric acid and heating the electrolyte during the electrolytic action to a temperature of approximately 95° F.

35 27. In the electrolytic refining of impure tin containing lead, the method of produc-

ing an appropriate electrolyte for the refining operation, which consists in passing an electric current at approximately 0.2 to 0.25 volts from the impure tin as an 40 anode to a cathode through an electrolyte capable of dissolving the tin in the anode while precipitating the lead and heating the electrolyte during the electrolytic tin 45 dissolving step.

28. In the electrolytic refining of impure 50 tin containing lead, the method of producing an appropriate electrolyte for the refining operation, which consists in passing an electric current at approximately 0.2 to 0.25 volts from the impure tin as an 55 anode to a cathode through an electrolyte capable of dissolving the tin in the anode while precipitating the lead and heating the electrolyte during the electrolytic tin dissolving step to a temperature of approximately 95° F.

29. In the electrolytic refining of impure 60 tin, the method of producing an appropriate electrolyte for the refining operation which consists in passing an electric current of relatively low voltage from the impure tin as an anode to a cathode through an electrolyte capable of dissolving the tin and subjecting the electrolyte to a temperature of approximately 95° F. during the 65 passage of the electric current.

Signed at Perth Amboy, in the county of Middlesex and State of New Jersey, this 10th day of December, A. D. 1920.

JAMES ROBERT STACK.